

Sept. 23, 1930.

M. C. FRANK

1,776,468

ASPHALTIC MATERIAL AND METHOD OF FABRICATION THEREOF

Filed Aug. 1, 1927



Fig. 1



Fig. 2



Fig. 3



Fig. 4



Fig. 5.



Fig. 6.



Fig. 8.

INVENTOR.



Fig. 7.

Maxwell C. Frank

## UNITED STATES PATENT OFFICE

MAXWELL C. FRANK, OF OAKLAND, CALIFORNIA

## ASPHALTIC MATERIAL AND METHOD OF FABRICATION THEREOF

Application filed August 1, 1927. Serial No. 209,727.

This invention relates especially to the use of asphaltic compositions as structural material for structures composed chiefly of asphaltic compositions.

5 It is primarily the object of my invention to improve the methods of utilization of asphalt to make its use as a structural material economically feasible.

10 It is an object of my invention to provide an improved method of fabricating asphaltic structures; and a further object, to provide an improved method of molding asphaltic material.

15 The immediate object of my invention is to provide an improved piping of asphaltic composition and method of making the same.

20 Other and ancillary objects of my invention will be suggested in the following description and in the uses to which my invention is put. Certain of the objects of my invention may be attained with the use of less than all its preferred features. It is desired that my invention be limited only by the claims constituting its final determination.

25 Referring to the drawings:

Fig. 1 is a median axial section of an apparatus for cold-molding asphaltic pipe segments; and Fig. 2 is a diametral section for the same. Certain elements are greatly exaggerated for the purpose of clarity.

30 Fig. 3 is a (transverse or longitudinal) section of a mold for cold-molding asphaltic bricks or slabs under solid compression instead of fluid pressure. A reinforced slab or brick is shown therein practically completed.

35 Fig. 4 is a fragmentary section of pipe showing a modified type of asphaltic concrete from that illustrated in Fig. 1, the same being reinforced.

40 Fig. 5 is a representation of a method of making and sealing a joint in the asphaltic piping of my invention.

45 Fig. 6 is a perspective representation of a flooring being fabricated of completely molded slabs, to illustrate the feature that the asphaltic slabs for road work (or for panelling), may be completely molded before

50 being laid.

Fig. 7 is a diagrammatic plan view of a form of apparatus for hot-forming asphalt slabs or bricks. Fig. 8 is a transverse section of the same; the plane of section being indicated by a line 9—9 in Fig. 7.

55 Asphalt heretofore has been limited largely to use as a surfacing or coating material, and has been practically limited to this use by its peculiar amorphous characteristic of "creeping." Asphalt is not a true solid. The creeping action is that of a highly viscous liquid which tends to conform to the surface on which it is placed. In order to adapt this material to structural purposes, I have provided a solid backbone of steel reinforcing. The steel in combination with asphalt is added primarily for elasticity and ability to hold the asphalt in shape, rather than for pure tensile strength as in hydraulic reinforced concrete. Examples of this reinforcing material (designated by the reference characters 1' and 1) are illustrated in Figs. 3 and 4. Preferably, the steel reinforcing should be a complete structure in itself and should be capable of resisting the

60 full value of the constantly-applied stresses plus the average value of the intermittent stresses, to which the combined asphalt and steel will be subjected. Since the intermittent stresses may occur infrequently and in

65 compensating directions, their average or mean value over an appreciable period of time is usually very slight. The very high viscosity of the asphaltic material insures

70 its resistance to all transitory stresses of short duration, and makes it especially resistant to suddenly-applied stresses. It has a deadening effect upon shock and vibration which practically insures the reinforcing framework against failure from this source.

75 This combination of a highly elastic material such as steel, with a highly viscous material such as asphalt, produces an especially valuable structural combination. In fabricating this material it will be noted from the drawings that a skeleton metal framework is preferred, and that it is found most advantageous to completely shroud the framework in the asphaltic material. The asphaltic material is preferably an asphaltic con-

55

60

65

70

75

80

85

90

95

100

crete essentially containing an asphalt, sand and rock aggregate in suitable proportions. If desired, some hydraulic cement may be added, and also other particles such as wood-fibres, straw, grass, cork, and the like.

Comparing this material to hydraulic concrete, two distinctions should be noted. The asphaltic material is not fragile and is especially resistant to shock. The asphaltic material is resistant to many of the acids which attack hydraulic concrete. The latter feature is especially important in the asphaltic pipe of my invention. The piping, segment of which is sectioned in Fig. 4, is formed of a porous steel skeleton cylindrical framework 1 of expanded metal sheet or other suitable skeleton section, shrouded in asphaltic concrete of relatively massive form; the asphaltic concrete constituting the major portion of the pipe, and the metal being only sufficient to hold the asphaltic material in shape and resist any slight constant loads which may be applied to it.

The asphaltic concrete is molded, either hot or cold, by any means preferred, and preferably under considerable compacting pressure, into pipe segments or sections, which are laid end-to-end or otherwise fabricated in the desired form, and are joined by merely applying localized heat to the joints as with a blowtorch. (See Figs. 6 and 7.) Where slabs, bricks, or other forms of the material are employed, of course the same principles apply. The completely molded forms are laid cold and are joined by heating only the joints.

Where the time factor is relatively unimportant, the joints may be permitted to seal themselves without the application of heat merely by the natural fluidity of the asphalt aided by gravity, pressure and wear, causing it to flow into the joints between segments. In general, this method of letting the joints seal themselves should be limited to the use of asphalt structural blocks where initial leakage past the new joints is not harmful.

The above features of my invention are unqualifiedly applicable to asphaltic structural elements whether formed hot by any of the methods well-known in the arts, or by a preferred hot-work method which I shall describe later, or by any cold-work method such as the preferred cold-work method I shall described.

The regular commercial grade of asphalt sold for paving work would require to be heated and molded hot. I have devised a method for molding the asphalt cold. Asphaltic emulsions such as "Laykold" are designed for surfacing purposes and my method permits their adaptation to molding. When these asphalt emulsions are spread or sprayed for surfacing purposes, evaporation is relied upon to remove the water content. I have

found it possible to remove the water content by pressure. The emulsion is poured or pumped into a mold (see Figs. 1 and 2), and the emulsifying agent is squeezed out under pressure. A design of one form of apparatus capable of accomplishing this method is illustrated by Figs. 1 and 2; and a modification thereof in Fig. 3.

For forming pipes, a concentric pair of heavy skeleton or apertured hollow cylinders 2 and 3 are telescoped to leave an annular molding space between. The cylinders are equal in length, and a pair of disk-shaped end caps 4 and 4' are removably held in place by an axial bolt 5 and nuts 6 and 7. The end plates may be provided with any suitable male and female means for forming on the ends of the pipe sections guiding and interlocking means for connecting them together, as for example, the tongue and groove 18 and 19 respectively; also, the end plates may be very slightly bowed (or finished to unequal thickness to give a bowed interior surface) so that the single bolt member will clamp the outer cylinder 2 as tightly as it does the inner cylinder 3. The inner cylinder 3 has a very finely porous thin plate 8 wrapped around it to prevent passage of asphalt from the mold when the emulsifying agent is being squeezed out. Similarly the outer cylinder 2 has a similar thin finely porous strainer plate 9 wrapped within it. A gate or inlet for the mold is conveniently formed by a pipe 10 threaded through a hole in one end cap 4. It is intended that the requisite molding pressure will be applied hydraulically by the pump 11 which fills the mold with the asphaltic concrete emulsion. Of course the pressure will be maintained for an appreciable interval of time to squeeze the material dry, and will be increased to finally compact or compress the mass.

The mold is stripped by removing one or both end caps, sliding out the finished pipe together with the two strainer plates 8 and 9, and then unwinding the two strainer plates to remove them.

A mold adapted to the formation of bricks, slabs, and other shapes is shown in Fig. 3. The body 12 of the mold is of heavy skeleton construction, and a removable strainer lining is formed by separate sheets 13, 13', 13'' etc. of thin finely porous metal similar to the strainer sheets 8 and 9. A skeleton plunger 14 completes the mold. Pressure is applied in this instance by a downward force upon the plunger 14; the mold being filled with asphaltic emulsion before the plunger is inserted.

In certain instances I have found it desirable to line the strainers with cloth; which may either be left on the molded product, or be stripped off and reused. Especially where the higher compacting pressures are employed, it frequently is advantageous to

use a small quantity of fibrous material in the asphaltic mix to form flow-lines along which the water may most readily be squeezed out.

5 A modified unapertured form of the mold illustrated in Fig. 8, forms the basis of an improved method of hot-forming asphalt, applicable especially to the large flat slabs of Fig. 7. The proportions of the mold would 10 of course be modified in accordance with the shape of slab to be formed, and the strainer plate 13, would be replaced by an unapertured stripper plate 15 extending longitudinally along the bottom of the mold and projecting up above the mold at one end thereof. The side-walls of the mold are reduced to the height of asphalt slab desired, and the piston 14 and strainer plate 13', 13" and 13 are dispensed with. The mold, after being 15 filled with the properly related layers of hot asphalt and steel skeleton structure, is passed under a battery of heavy rolls 16 which ride on the top edge of the mold, and compact the asphalt much as would a steam roller of the 20 type commonly used in street paving work. Satisfactory rolls for the purpose may be appropriated from, and are well-known in the steel rolling or paper industries. To form 25 bricks by this method it is simply necessary 30 to place properly-spaced divider plates 17 in a long channel-like mold. The divider plates may be of sheet metal or other impervious material, merely to prevent adhesion between adjacent bricks. To strip the mold it is 35 merely necessary to pull the exposed end 15' of the stripper plate 15.

I claim:

1. The method of forming a solid article of asphaltic concrete which comprises placing cold fluid asphaltic concrete forming material having the asphalt thereof emulsified in a mold and thereafter uniformly expressing the emulsifying liquid through the mold walls to free the asphalt for adhesive union with the other elements of said material.
2. The method of forming an asphaltic body which comprises the steps of placing a mixture containing asphaltic emulsion in a mold, and demulsifying the emulsion entirely by compression of the said mixture in said mold.
3. The method of forming an asphaltic body which comprises the steps of placing a mixture containing asphaltic emulsion in a mold, and demulsifying the emulsion in place.
4. The method of forming an asphaltic concrete which comprises the steps of placing a generally non-cohesive mixture containing asphaltic emulsion in a mold, and demulsifying the emulsion in place in said mold and at a normal temperature.
5. The method of forming an asphaltic body which comprises pressure-molding a

mixture containing asphaltic emulsion while said mixture is at a normal temperature.

6. The method of producing an artificial concrete of a normally adhesive and emulsifiable binder material and particles of other and solid material, which comprises the steps of emulsifying said first material, forming a homogeneous mixture of the resulting emulsion and said second material, and pressure-molding said mixture to demulsify said binder material therein for adhesive union with the second material.

7. The method of producing an artificial concrete of a normally adhesive and emulsifiable binder material and particles of other and solid material, which comprises the steps of emulsifying said first material, forming a homogeneous mixture of the resulting emulsion and said second material, and demulsifying said first material in the mixture by pressure and at a normal temperature whereby to produce a cohesive mass of said materials.

In testimony whereof, I affix my signature.

MAXWELL C. FRANK.

90

95

100

105

110

115

120

125

130

70

75

80

85

90

100

105

110

115

120

125

130